

# United States Patent [19]

Vander Wall et al.

[11] 3,751,311

[45] Aug. 7, 1973

[54] GELATION OF HYDRAZINE AND  
HYDRAZINE-TYPE ROCKET FUELS

[75] Inventors: Eugene M. Vander Wall, Citrus  
Heights; James M. Lucas, El Dorado  
Hills, both of Calif.

[73] Assignee: Aerojet-General Corporation, El  
Monte, Calif.

[22] Filed: July 27, 1967

[21] Appl. No.: 658,982

[52] U.S. Cl. .... 149/36, 49/20

[51] Int. Cl. .... C06c 1/02

[58] Field of Search .... 149/17, 18, 36, 20

## [56] References Cited

### UNITED STATES PATENTS

3,077,072 2/1963 Rice .... 149/36

|           |        |                              |
|-----------|--------|------------------------------|
| 3,164,505 | 1/1965 | Hsieh et al. .... 149/36     |
| 3,196,059 | 7/1965 | Godfrey .... 149/36 X        |
| 3,197,348 | 7/1965 | Skolnik et al. .... 149/36 X |
| 3,232,801 | 2/1966 | Bost et al. .... 149/36 X    |

Primary Examiner—Carl D. Quarforth

Assistant Examiner—Stephen J. Lechert, Jr.

Attorney—Edward O. Ansell, D. Gordon Angus and  
Donald W. Grauer

[57]

## ABSTRACT

This patent describes novel gelled hydrazine-type fuels suitable for use in rockets, missiles and the like. The gelling agents are quaternary ammonium salts of polyacrylic acid.

7 Claims, No Drawings

## GELATION OF HYDRAZINE AND HYDRAZINE-TYPE ROCKET FUELS

### BACKGROUND OF THE INVENTION

The field of the present invention pertains to gelled rocket fuels.

Various hydrazine-type fuels are well known for use in liquid rocket engines. However, liquid hydrazine-type materials are characterized by several problems. One of these is the tendency to slosh within fuel tanks during flight. Sloshing has been found to adversely affect the stability of the rocket. Liquid hydrazine fuels also present a safety hazard since they can easily escape through ruptured or perforated tanks or fuel lines. For these and other reasons, various gelling agents have been proposed to thicken or produce a mechanically stable gel of hydrazine. One example of such a gelling agent is polyacrylic acid which is disclosed in assignees' U.S. Pat. No. 3,232,801 issued Feb. 1, 1966. This patent describes the use of polyacrylic acid as a gelling agent to produce a mechanically stable, thixotropic hydrazine-type gel. The compositions of this patent are quite satisfactory in most respects. However, certain significant improvements have now been discovered and the present patent application is directed to these improvements.

### SUMMARY OF THE INVENTION

Briefly, the present invention comprises a gelled, mechanically stable, thixotropic liquid fuel composition comprising a hydrazine-type fuel containing an effective gelling amount of a gelling agent which is a quaternary ammonium salt of polyacrylic acid. The invention further comprises a method of preparing novel gelled fuel compositions.

As has been indicated above, it is desirable to gel rocket fuels so that the liquid is immobilized to reduce seepage and leakage hazards, and prevent sloshing of the liquid in propellant tanks. It is also desirable to gel rocket fuels so that solid energetic particles, usually solid metals, can be permanently and uniformly suspended in the fuels to increase the fuel value. Gelation also aids in holding the propellant in its position in fuel tanks under conditions of 0 gravity. The quaternary ammonium salts of the present invention are superior to known gelling agents in that at concentration levels of less than 5 percent, they will gel fuels that cannot be gelled by the incorporation of ordinary polyacrylic acid. The quaternary ammonium salts of the present invention can also be used to gel several different types of hydrazine-type fuels and are not restricted in their use to the gellation of ordinary hydrazine or hydrazine-containing mixtures.

The gels of the present invention are also less sensitive to ionic contamination than are other polymers used for gelation. The hydrazine gels of the present invention have been found to be stable over a greater temperature range than hydrazine gelled with polyacrylic acid. Further, the gelling agents of the present invention can be completely neutralized so that no acidic species are introduced into the fuels, making the fuels less reactive with acid-sensitive metals and compounds.

Accordingly, it is a principal object of the present invention to provide a mechanically stable, thixotropic gelled hydrazine-type fuel composition.

Another object of the present invention is to provide a means of gelling hydrazine-type fuel compositions having a wider applicability than has previously been available.

Still another object of the present invention is to provide a gelled hydrazine fuel composition which is stable over a greater temperature range than known gelled hydrazines.

It is still another object of the present invention to provide a gelled hydrazine-type fuel which is less sensitive to ionic contamination.

A further object of the present invention is the provision of a gelled fuel composition which is less reactive with acid-sensitive metals and other fuel additives.

These and other objects and advantages of the present invention will become apparent from a more detailed description which follows.

### DESCRIPTION OF THE PREFERRED EMBODIMENTS

The gelling agents of the present invention are normally employed in effective gelling amounts up to about 10 percent by weight of the total fuel composition. However, it should be understood that even greater amounts of the gelling agent may be employed, although this is normally to be avoided since the gelling agents are completely effective at low concentration and the use of more gelling agent is of no further benefit.

There may be included in the gelled hydrazine-type fuels of the present invention, as an optional ingredient, powdered metals such as aluminum or beryllium. These metals serve to increase the specific impulse of the fuel. The amount of powdered metal employed is not critical. Normally, if the powdered metal is added, it should be used in amounts up to about 60 percent by weight of the total weight of the gelled fuel compositions. When these metals are incorporated in the gelled hydrazine compositions, it has been found that the resulting fuel is mechanically stable and there is no tendency for the powdered metal to settle out of the gel.

The quaternary ammonium polyacrylate salts used as the gelling agents of the present invention are prepared by neutralizing a suitable polyacrylic acid with a quaternary ammonium hydroxide in a solvent. The solvent is removed after neutralization and the salt is dried in vacuum at room temperature.

The amount of quaternary ammonium hydroxide used may be enough to neutralize all of the free carboxyl groups in the polyacrylic acid. However, in many cases, less than a stoichiometric amount of quaternary ammonium hydroxide is used. The use of partially neutralized polyacrylic acid has been found to reduce the quantity of a gelling agent which is required for gellation compared to that required when the completely neutralized salt is used. In other cases where acid-sensitive metals or other additives are to be employed, it has been found that it is preferred to employ a completely neutralized gelling agent which introduced no acidic species into the fuels. Thus, based upon the foregoing criteria, those skilled in the art will be able, within the scope of the present invention and in accordance with the teachings of this patent, to select a gelling agent to provide optimum gelation in each specific fuel composition while minimizing the amount of gelling agent required.

The following examples are presented solely to illustrate the invention and should not be regarded as limiting in any way. In the examples, the parts and percentages are by weight unless otherwise indicated.

## EXAMPLE 1

The following example illustrates the preparation of the gelling agent of the present invention. 5.42 grams (0.72 equivalents) of suitable polyacrylic acid, Car-

tetrapropyl ammonium hydroxide in the above example, tetramethyl ammonium polyacrylate and tetraethyl ammonium polyacrylate were obtained.

## EXAMPLE 2

The quaternary ammonium polyacrylate salts prepared as indicated above were dispersed in a hydrazine-type fuel to produce gels. The characteristics of the gel and their composition are shown in the following table.

TABLE I

| Polyacrylate gelling agent           | Components of gels         |                                                                                                       | Physical properties                                        |                         |
|--------------------------------------|----------------------------|-------------------------------------------------------------------------------------------------------|------------------------------------------------------------|-------------------------|
|                                      | Gellant conc.<br>(percent) | Fuel                                                                                                  | High shear viscosity<br>(cp.) (17,300 sec. <sup>-1</sup> ) | Gel is stable to—(° F.) |
| Tetramethyl-ammonium                 | 1.37                       | Hydrazine                                                                                             | 37                                                         | >165                    |
| Tetraethyl-ammonium                  | 1.83                       | do                                                                                                    | 30                                                         | >165                    |
| Tetrapropyl-ammonium                 | 1.40                       | do                                                                                                    | 26                                                         | >165                    |
| Tetrachethyl-ammonium                | 8.1                        | Monomethyl hydrazine                                                                                  | 34                                                         | —                       |
| Tetrapropyl-ammonium                 | 4.1                        | do                                                                                                    | 24                                                         | >165                    |
| Tetrapropyl-ammonium 34% neutralized | 2.0                        | do                                                                                                    | 23                                                         | 133                     |
| Tetrapropyl-ammonium                 | 3.7                        | {14% hydrazine<br>188% monomethyl hydrazine<br>50% hydrazine<br>50% unsymmetrical dimethyl hydrazine} | 33                                                         | >212                    |
| Do                                   | 2.6                        | {50% unsymmetrical dimethyl hydrazine}                                                                | 35                                                         | —                       |

bopol-940, a polyacrylic acid manufactured by B. F. Goodrich Company, are dispersed in 550 ml of methanol. As this solution is stirred, 142 grams of a 10 percent aqueous solution of tetrapropyl ammonium hydroxide (0.072 equivalents) available from Eastman Chemical Products Company are gradually added. The entire addition requires five minutes. A gel forms, and stirring is continued for two hours to assure complete mixing. Methanol and water are removed by evaporation under vacuum. The product is vacuum-dried at a pressure of 5 mm Hg for four days at room temperature. The product is a glass-like material which requires grinding to facilitate dispersal in liquids. The yield is 19 grams of tetrapropyl ammonium polyacrylate which corresponds to 97 percent of the theoretical yield. Losses are primarily incurred in handling. The pH of an 0.01 N solution of tetrapropyl ammonium polyacrylate in water is 8.8. The equivalent weight of this salt is 260.

By substituting tetramethyl ammonium hydroxide and tetraethyl ammonium hydroxide, respectively, for

The hydrazine gels prepared with quaternary ammonium salts do not break down upon prolonged exposure to the atmosphere, while hydrazine gels prepared with the polyacrylic acid itself break down upon brief exposure.

The following tables illustrate the properties of various gels within the scope of this invention.

TABLE II.—PROPERTIES OF HYDRAZINE GELS PREPARED WITH VARIOUS GELLING AGENTS

| Gelling agent                     | Gelling agent, percent | High shear viscosity, cp. | Yield stress, dynes/cm. <sup>2</sup> | Gel breakdown temperature, ° F. |
|-----------------------------------|------------------------|---------------------------|--------------------------------------|---------------------------------|
| Tetramethyl ammonium polyacrylate | 0.94                   | 25                        | 600                                  | >165                            |
| Do                                | 1.47                   | 64                        | 2,800                                | >165                            |
| Tetrapropyl ammonium polyacrylate | 1.40                   | 26                        | (*)                                  | >165                            |
| Do                                | 1.88                   | 46                        | 600                                  | >165                            |
| Tetrabutyl ammonium acrylate      | 2.92                   | 14                        | 300                                  | (*)                             |

\*Property not determined.

TABLE III.—PROPERTIES OF METALIZED HYDRAZINE GELS

| Gelling agent                                     | Composition |        | Yield stress, dynes/cm. <sup>2</sup> | High shear viscosity, cp. | Gel-liquid transition temperature, ° F. |
|---------------------------------------------------|-------------|--------|--------------------------------------|---------------------------|-----------------------------------------|
|                                                   | Percent     | Metal  |                                      |                           |                                         |
| Tetramethyl ammonium polyacrylate                 | 0.58        | 43% Al | 1,300                                | 50                        | >160                                    |
| Do                                                | 0.48        | 43% Al | (*)                                  | 30                        | >160                                    |
| Tetramethyl ammonium polyacrylate 50% neutralized | 0.48        | 43% Al | (*)                                  | 48                        | >160                                    |
| Tetrapropyl ammonium polyacrylate                 | 1.27        | 43% Al | 1,200                                | 52                        | >160                                    |
| Do                                                | 0.58        | 43% Al | (*)                                  | 28                        | >160                                    |
| Do                                                | 0.91        | LM-2   | 1,000                                | 39                        | >160                                    |

\*Property not determined.

TABLE IV.—PROPERTIES OF HYDRAZINE-TYPE FUELS GELLED WITH POLYACRYLATE GELLING AGENTS

| Gelling agent                     | Fuel                 | Gelling agent concentration, percent | High shear viscosity, cp. | Yield stress, dynes/cm. <sup>2</sup> | Gel stability temperature limits, °F. |
|-----------------------------------|----------------------|--------------------------------------|---------------------------|--------------------------------------|---------------------------------------|
| Tetraethyl ammonium polyacrylate  | Monomethyl hydrazine | 8.1                                  | 34                        | (*)                                  | (*)                                   |
| Tetrapropyl ammonium polyacrylate | do                   | 4.0                                  | 20                        | 100                                  | <-65, >165                            |
| Do                                | do                   | 8.6                                  | 67                        | 2,200                                | <-65, >165                            |
| Tetrabutyl ammonium polyacrylate  | do                   | 2.9                                  | 16                        | (*)                                  | <-65, >165                            |

\*Property not determined.

In general, it can be seen from the foregoing examples that the stable hydrazine gels of this invention are produced by mixing a gelling agent with hydrazine. It is to be understood that powdered metals such as powdered aluminum, can be blended either before, after, or along with the gelling agent. The ingredients are normally blended by shaking or by mechanical agitation to uniformly distribute the gelling agent and to deagglomerate the powdered metal.

The significant improvement in the gel stability in the presence of ions is shown by the comparative data on the following table.

TABLE V.—EFFECT OF SODIUM NITRATE (ION) CONCENTRATION ON THE HIGH SHEAR VISCOSITY OF HYDRAZINE GELLED WITH SALTS OF POLYACRYLIC ACIDS

| Polyacrylic acid            |                                      |                 | Monomethylhydrazonium salt of polyacrylic acid |                                      |                 |
|-----------------------------|--------------------------------------|-----------------|------------------------------------------------|--------------------------------------|-----------------|
| Gellant concentration (W/O) | Sodium nitrate (p.p.m.) <sup>3</sup> | Viscosity (cp.) | Gellant concentration (W/O)                    | Sodium nitrate (p.p.m.) <sup>3</sup> | Viscosity (cp.) |
| 0.66                        | 0                                    | 27.8±1.0        | 0.70                                           | 0                                    | 21.4±1.0        |
| 0.66                        | 52                                   | 17.4±0.5        | 0.67                                           | 51                                   | 13.4±0.0        |
| 0.66                        | 93                                   | 12.6±1.1        | 0.67                                           | 84                                   | 11.0±0.4        |
| 0.66                        | 200                                  | 9.7±0.3         | 0.67                                           | 194                                  | 9.2±1.5         |
| 0.66                        | 286                                  | 7.1±0.7         |                                                |                                      |                 |

#### TETRAPROPYLAMMONIUM SALT OF POLYACRYLIC ACID

| Gellant concentration (W/O) | Sodium nitrate (p.p.m.) <sup>3</sup> | Viscosity (cp.) |
|-----------------------------|--------------------------------------|-----------------|
| 1.40                        | 0                                    | 26.0±1.2        |
| 1.33                        | 51                                   | 23.1±0.8        |
| 1.33                        | 98                                   | 19.5±1.2        |
| 1.33                        | 337                                  | 16.6±0.2        |

NOTE.—All viscosity measurements are reported at a shear rate of 17,300 sec.<sup>-1</sup>.

While the present invention has been specifically illustrated with hydrazine monomethyl hydrazine and unsymmetrical dimethyl hydrazine, it is to be understood that it is applicable to all types of hydrazine-type fuels, including mixtures of various hydrazine-type fuels.

The gelled fuels of the present invention are highly energetic and are directly useful as fuels in liquid rocket motors.

As can be seen from the foregoing discussion, the gelled fuels of the present invention can be made quite insensitive to acidic reacting liquid propellant additives. The gels of this invention are also stable over a wide range of temperatures. In addition, the gelling agents employed in the present invention can be varied in accordance with the particular fuel to be gelled. Thus, if the fuel is to contain an acid-reacting ingredient, the gelling agent can be completely neutralized. On the other hand, if no acid-reacting additive is to be employed, then, the gelling agent need only be partly neutralized, and in this case the amount of gelling agent required can be reduced. It is therefore apparent that the present invention will find wide application in the space and defense missile efforts.

Having fully described the invention, it is intended that it be limited only by the lawful scope of the appended claims.

We claim:

1. A gelled mechanically stable thixotropic high-energy fuel composition comprising a hydrazine-type fuel selected from the group consisting of hydrazine and alkyl substituted hydrazines containing therein an effective gelling amount of a gelling agent comprising a quaternary ammonium salt of polyacrylic acid.
2. The composition of claim 1 wherein the gelling agent is tetramethyl ammonium polyacrylate.
3. The composition of claim 1 wherein the gelling agent is tetraethyl ammonium polyacrylate.
4. The composition of claim 1 wherein the gelling agent is tetrapropyl ammonium polyacrylate.
5. The composition of claim 1 wherein the gelling agent is tetrabutyl ammonium polyacrylate.
6. The composition of claim 1 wherein the gelling agent comprises a partially neutralized quaternary ammonium salt of polyacrylic acid.
7. The composition of claim 1 wherein there is additionally present finely divided metal fuel in an amount up to about 60 percent by weight of the composition.

\* \* \* \* \*